

## UNITED STATES PATENT OFFICE

2,303,399

## ALKALINE DETERGENT

Charles Schwartz, Pittsburgh, Pa., assignor to  
 Hall Laboratories, Inc., Pittsburgh, Pa., a corporation of Pennsylvania

No Drawing. Application May 1, 1939,  
 Serial No. 271,178

11 Claims. (Cl. 252—135)

This invention relates generally to alkaline preparations, for example alkaline detergents for cleaning soft metals and more particularly to such detergents containing alkali-metal silicates and an inhibiting agent for preventing the alkaline corrosion of the metal.

It is a well known fact that many highly alkaline detergents while performing excellently as cleaners can not be used for the cleaning of soft metals such as aluminum and tin, since the alkalies corrode and dissolve the metals quite readily.

Many efforts have been made to utilize the excellent detergent properties of highly alkaline mixtures and at the same time to prevent, in so far as possible, the attack upon soft metals. Thus the use of certain silicates has been successful in decreasing to a considerable extent the corrosion of aluminum in alkaline solutions. It is necessary, however, to be very careful in the choice of silicate used and in the concentration of the solution in order to avoid very serious attack upon the metal being washed. If the concentration of the solution is too high or too low, it attacks the aluminum and this places a serious limitation on the type of solution which may be employed.

Silicates have been used also for cleaning tin but in this case the alkalinity of the cleaning solution must be adjusted to so low a pH and the temperature of cleaner dropped to such an extent that effective cleaning can not easily be obtained. Other remedies for the corrosion of tin and aluminum by alkaline cleaners have been suggested also. In the case of tin, the use of sodium sulphite has become quite widespread in recent years. This material decreases the oxygen concentration of the cleaning solution and inhibits the corrosion of tin by alkalies. However, there is considerable corrosion after the sulphite is depleted, as it is very shortly in usual practice. Where the solution is heated in contact with air, the sodium sulphite is readily converted into sodium sulphate, which is ineffective in preventing corrosion.

Probably the most successful remedy for corrosion which has been found thus far has been the addition of chromates or dichromates to alkaline materials in the washing of soft metals. While in general these materials are quite successful in preventing corrosion, they have two serious drawbacks. They tend to coat the metal being washed with a greenish yellow film which in most cases is very undesirable. Most people are sensitive to chromates and the operators using the cleaners frequently suffer from what

is known as "chromic ulcers," which necessitate cessation of all work with material containing chromates and which require long periods of time for healing.

It is an object of the present invention to provide means by which alkaline detergents may be made safe for cleaning soft metals. The present invention has many advantages over the methods previously employed. Aluminum, tin, zinc, lead, cadmium or other soft metals thereof may be treated with solutions of extremely high pH at boiling temperatures for long periods of time without showing any evidence of corrosion. The cleaning solutions preferably have a pH of at least 10 and in many cases the pH is as high as 12 or over. The corrosion inhibitors which I employ do not decrease in effectiveness with time, as do the sulphites, but remain effective over long periods. They are without harmful effect upon the human skin and will not occasion the difficulties accompanying the use of chromates or dichromates.

I have found that the water-soluble salts of arsenic and antimony when added in proper proportion to alkali-metal silicates or to a mixture of alkalies containing an alkali-metal silicate as its principal alkaline ingredient prevent entirely the characteristic corroding effect of these silicates. The mechanism whereby the corrosion is prevented is unknown but it probably can be ascribed to the formation of non-reactive protective films on the metal surfaces.

Sodium metasilicate, sesquisilicate and orthosilicate are strong alkalies, their alkalinity increasing in the order listed. It is well known that even the weakest of these, namely sodium metasilicate when used for example to wash tin or tin plate causes rapid spangling and solution of the tin even at relatively low temperature. I have found that by adding a small quantity of a water-soluble arsenic or antimony salt to any of these silicates the corrosive effect of the solution subsequently made from it is reduced to zero even at boiling temperatures over long periods of time.

Although I prefer to use the chlorides of arsenic or antimony as the water-soluble salts which inhibit corrosion of the soft metals, I may employ any ordinarily water-soluble salt, such as arsenic iodide, fluoride, or antimony fluoride or tartrate. The amount of water-soluble arsenic or antimony salts required for preventing corrosion will depend upon the metal to be treated, the treating solution and the conditions of treatment. Under most conditions, I prefer

to use at least 5% of arsenic salt based on the weight of the alkali with which it is used. If an antimony salt is employed, it is necessary to use somewhat more than in the case of arsenic. The minimum amount of antimony salt is in the neighborhood of 10%, based on the weight of the alkali with which it is used. I have found that about 15-20% of antimony chloride (based on the weight of the sodium metasilicate) is required to entirely prevent the corrosion of tin by a 1% solution of sodium metasilicate at boiling temperatures. Under the same conditions, I have found that about 5-10% of arsenic chloride is required to inhibit the corrosion of tin appreciably, although the corrosion is not completely prevented by this material. Under less severe conditions, less of the arsenic or antimony salts may be employed and it will be understood that these salts may be used in amounts above those mentioned without harmful effect, although this is usually unnecessary.

The preferred alkaline material for use in preparing the alkaline detergent solutions are the alkali-metal silicates, such, for example, as the metasilicates, sesquisilicates and orthosilicates; although the alkalinity of the solutions prepared therefrom may be increased by adding sodium hydroxide or other strong alkali. Particularly in the case where antimony is used as the inhibiting salt, it is preferred that the detergent contain an alkali-metal silicate as its principal alkaline ingredient. The inhibiting effect of the antimony is greater in such cases than where the detergent is composed primarily of some other alkali than an alkali-metal silicate.

In the case of arsenic inhibiting salts, although I prefer that they be used with alkalies containing alkali-metal silicate as their principal alkaline ingredient, they inhibit the corrosive effects of phosphates, carbonates, silicates or their combinations with each other, with or without the addition of sodium hydroxide or other strong alkali.

The water-soluble arsenic or antimony salts act as inhibitors in the presence of mixtures of silicates with sodium hydroxide or other alkalies, soap, casein, deflocculating agents, wetting agents, abrasives and the like.

The alkaline solution containing the corrosion inhibitor is useful in all cases where a highly alkaline detergent is required. It may be used for example in the washing of tin plates, tubes, bakery pans, milk cans, and in tin fabricating plants. In the fabrication of tin plate, or articles made therefrom, it is often necessary to apply grease to aid in the forming operations. This may be removed by the use of a highly alkaline cleaning solution in accordance with the present invention without attack on the tin. The cleaning solutions may be used also in the treatment of aluminum. In this case also, the solution may be used to remove the grease employed in fabricating the aluminum without, however, causing alkaline corrosion of the aluminum.

For washing pans in a bakery where the pans are washed fairly frequently, so that the amount of burned on matter is not excessive, I may use a cleaning composition containing about 95% sodium metasilicate and 5% of arsenic or antimony chloride or other water-soluble salts of these metals. This is dissolved in water to form a solution of a strength between  $\frac{1}{4}$  of 1% and 3%, usually about 1%. The pans might be boiled in the cleaning solution for an hour.

Where the deposits on the bakery pans are excessive, I might use an aqueous solution of a composition containing 95% sodium orthosilicate and 5% of an inhibiting arsenic or antimony salt.

As another example, I might use a 1% aqueous solution of a composition containing 60% sodium metasilicate, 35% sodium hydroxide and 5% of arsenic or antimony chloride or other water-soluble salt of these metals. I might add to this or to any of the compositions a wetting agent such as a sodium salt of a sulphated fatty alcohol in the amount of 1-3% based on the total weight of the solids. In addition, I might add soap, casein, deflocculating agents, wetting agents, abrasives and the like.

The invention enables the use of highly alkaline solutions containing alkali-metal silicates or other strong alkalies in the cleaning of soft metals without corrosion of the metal. It is preferred that the aqueous solution of the detergent composition have a pH of at least 10 and in many cases it is 12 or over. Thus powerful cleaners may be prepared which by reason of their speed of cleaning, non-corrosiveness and other features referred to are superior to any products now available. Although the invention will probably find its greatest use in connection with preventing the corrosion of aluminum and tin, it is applicable also to the treatment of zinc, lead, cadmium or other soft metals or alloys thereof. The term "soft metal" as used herein is intended to include any metal or alloy which under the proper conditions of temperature and concentration tends to be attacked or dissolved by alkaline solutions.

Although the principal use of the invention is in connection with cleaning solutions, the invention is applicable to inhibiting corrosion by alkaline compositions in general and silicate containing compositions in particular, as for example by the use of such compositions as paints or adhesives. The addition of a water-soluble salt of arsenic or antimony to a silicate containing paint or adhesive will prevent the attack of the paint or adhesive on soft metals, during the time required for the paint or adhesive to set or harden.

The invention is not limited to the examples, which have been given merely for illustrative purposes, or to the preferred proportions, but may be otherwise embodied or practiced within the scope of the following claims.

I claim:

1. An alkaline detergent composition for soft metal, comprising an alkali-metal silicate as its principal alkaline ingredient and being of such character that under normal conditions of use it will corrode the soft metal, and a water-soluble arsenic salt in an amount of at least 5% based on the weight of the alkali-metal silicate to inhibit corrosion of the soft metal.

2. An alkaline detergent composition for soft metal, comprising an alkali-metal silicate as its principal alkaline ingredient and being of such character that under normal conditions of use it will corrode the soft metal, and a water-soluble antimony salt in an amount of at least 10% based on the weight of the alkali-metal silicate to inhibit corrosion of the soft metal.

3. An alkaline detergent composition for soft metal, comprising by weight about 95% sodium metasilicate and about 5% water-soluble salt of a metal of the group consisting of arsenic and antimony.

4. An alkaline detergent composition for soft metal, comprising by weight about 95% sodium metasilicate and about 5% of a chloride of metal of the group consisting of arsenic and antimony.

5. An alkaline detergent composition for soft metal, comprising by weight about 95% sodium orthosilicate and about 5% of water-soluble salt of a metal of the group consisting of arsenic and antimony.

6. An alkaline detergent composition for soft metal, comprising by weight about 95% sodium orthosilicate and about 5% of a chloride of metal of the group consisting of arsenic and antimony.

7. An alkaline detergent composition for soft metal, comprising by weight about 60% sodium metasilicate, about 35% sodium hydroxide and about 5% of water-soluble salt of a metal of the group consisting of arsenic and antimony.

8. An alkaline detergent composition for soft metal, comprising by weight about 60 to 95% sodium metasilicate, an effective amount up to about 35% sodium hydroxide, and about 5 to 20% water-soluble salt of a metal of the group consisting of arsenic and antimony.

9. An alkaline detergent composition for soft metal, comprising an alkali-metal silicate as its principal alkaline ingredient and being of such character that under normal conditions of use it will corrode the soft metal, and an effective

amount of a water-soluble salt of a metal of the group consisting of arsenic and antimony to inhibit the corrosion of the soft metal, an effective amount being at least 5% in the case of the arsenic salt and at least 10% in the case of the antimony salt, based on the weight of said alkali-metal silicate.

10. An alkaline detergent composition for soft metal having a pH of at least 10 in aqueous solution and being of such character that under normal conditions of use it will corrode the soft metal, said detergent composition comprising an alkali-metal silicate as its principal alkaline ingredient, and an effective amount of a water-soluble salt of a metal of the group consisting of arsenic and antimony to inhibit the corrosion of the soft metal, an effective amount being at least 5% in the case of the arsenic salt and at least 10% in the case of the antimony salt, based on the weight of said alkali-metal silicate.

11. An alkaline detergent composition for soft metal, comprising by weight about 60 to 95% sodium metasilicate, an effective amount up to about 35% of an alkali-metal salt having a higher alkalinity than sodium metasilicate, and about 5 to 20% water-soluble salt of a metal of the group consisting of arsenic and antimony.

CHARLES SCHWARTZ.